# EUROPEAN PATENT APPLICATION

(11) **EP 1 176 029 A2**
(43) Date of publication of application: **30.01.2002**
(21) Application number: 01202701.7
(22) Date of filing: 16.07.2001
(51) Int. Cl.: B41M 5/00

(54) **Ink jet recording element and printing method**

(30) Priority: 27.07.2000 US 626752; 27.07.2000 US 627052
(71) Applicant: EASTMAN KODAK COMPANY, Rochester, New York 14650 (US)
(72) Inventor: Landry-Coltrain, Christine, c/o Eastman Kodak Comp, Rochester, New York 14650-2201 (US); Teegarden, David M., c/o Eastman Kodak Company, Rochester, New York 14650-2201 (US); Franklin, Linda M., c/o Eastman Kodak Company, Rochester, New York 14650-2201 (US); Hoffman, Christopher R., c/o Eastman Kodak Company, Rochester, New York 14650-2201 (US)
(74) Representative: Nunney, Ronald Frederick Adolphe

(57) **Abstract**

An ink jet recording element comprising a support having thereon an image-receptive layer capable of accepting an ink jet image comprising an open-pore membrane of a mixture of a water-insoluble polymer and a water-absorbent polymer, the mixture containing at least 25% by weight of the water-absorbent polymer, the image-receiving layer being made by dissolving the mixture of polymers in a solvent mixture, the solvent mixture comprising at least one solvent which is a good solvent for the water-insoluble polymer and at least one poor solvent for the water-insoluble polymer, the poor solvent having a higher boiling point than the good solvent, coating the dissolved mixture on the support, and then drying to remove approximately all of the solvents to obtain the open-pore membrane.

## Description

This invention relates to an ink jet recording element, more particularly to a porous ink jet recording element and a printing method.

In a typical ink jet recording or printing system, ink droplets are ejected from a nozzle at high speed towards a recording element or medium to produce an image on the medium. The ink droplets, or recording liquid, generally comprise a recording agent, such as a dye or pigment, and a large amount of solvent. The solvent, or carrier liquid, typically is made up of water, an organic material such as a monohydric alcohol, a polyhydric alcohol or mixtures thereof.

An ink jet recording element typically comprises a support having on at least one surface thereof an ink-receiving or image-forming layer. The ink-receiving layer may be a porous layer which imbibes the ink via capillary action or a polymer layer which swells to absorb the ink.

Ink jet prints, prepared by printing onto ink jet recording elements, are subject to environmental degradation. They are especially vulnerable to water smearing and light fade. For example, since ink jet dyes are water-soluble, they can migrate from their location in the image layer when water comes in contact with the receiver after imaging. Highly swellable hydrophilic layers can take an undesirably long time to dry, slowing printing speed, and will dissolve when left in contact with water, destroying printed images. Porous layers speed the absorption of the ink vehicle, but often suffer from insufficient gloss and severe light fade. Porous layers are also difficult to coat without cracking.

U.S. Patent 4,849,457 discloses a porous membrane for use as a recording medium for ink jet printing comprising a mixture of two water-insoluble polymers and 9% of polyvinylpyrrolidone. However, there is a problem with this element in that the density obtained with an element having less than 25% by weight of a water-absorbent polymer is too low, as will be shown hereafter. Further, this membrane is made by coating the two materials from a solvent, and then passing the coated element through a nonsolvent bath. The porous membrane employed in this invention is formed solely upon drying of the coated solution without the need for a nonsolvent bath.

JP95040647A discloses a porous membrane for use as a recording medium for ink jet printing comprising a mixture of a hydrophobic binder containing cationic conductive macromolecules. However, there is a problem with this element in that the density and dye lightfastness obtained with an element having less than 25% by weight of a water-absorbent polymer is too low, as will be shown hereafter.

U.S. Patent 5,374,475 discloses a porous layer for ink jet printing comprising a thermoplastic polymer free of filler. However, there is a problem with this element in that the density obtained with an element without a water-absorbent polymer is too low, as will be shown hereafter.

U.S. Patent 5,759,639 discloses a printing medium for ink jet printing which uses a polymeric dope solution. A porous layer is formed using a phase inversion technique. Although a second polymer is used in the process, most of it is washed out in a coagulation step. There is a problem with this element in that the density obtained with an element having less than 25% by weight of a water-absorbent polymer is too low, as will be shown hereafter.

EP 940,427 discloses a method for making a microporous film for an ink jet recording element in which a hydrophobic polymer and a second hydrophilic polymer or copolymer of N-vinylpyrrolidone is dissolved in a certain solvent system, partially dried, and then washed to extract at least 50% by weight of the second polymer. There is a problem with the elements formed by this process in that a separate washing step is employed which adds to the complexity of the coating process.

It is an object of this invention to provide an ink jet recording element which will provide improved ink uptake speed. Another objective of the invention is to provide an ink jet recording element having a receiving layer that when printed upon has an excellent image quality. Another object is to provide an ink jet printing method.

These and other objects are provided by the present invention comprising an ink jet recording element comprising a support having thereon an image-receptive layer capable of accepting an ink jet image, said layer comprising an open-pore membrane of a mixture of a water-insoluble polymer and a water-absorbent polymer, the mixture containing at least 25% by weight of the water-absorbent polymer, the image-receiving layer being made by dissolving the mixture of polymers in a solvent mixture, the solvent mixture comprising at least one solvent which is a good solvent for the water-insoluble polymer and at least one poor solvent for the water-insoluble polymer, the poor solvent having a higher boiling point than the good solvent, coating the dissolved mixture on the support, and then drying to remove approximately all of the solvents to obtain the open-pore membrane.

Using the invention, a recording element is obtained which will provide improved ink uptake speed and when printed upon has an excellent image quality.

Another object of the invention relates to an ink jet printing method comprising the steps of:
A) providing an ink jet printer that is responsive to digital data signals;
B) loading the printer with an ink jet recording element as described above;
C) loading the printer with an ink jet ink composition; and
D) printing on the ink jet recording element using the ink jet ink in response to the digital data signals.

In order for the image-receptive layer to be sufficiently porous, the water-insoluble polymer must be coated from a solvent mixture combination such that an open-pore membrane structure will be formed when the solution is coated and dried, in accordance with the known technique of dry phase inversion. The formation of an open-pore membrane is accomplished by using a mixture of a good and poor solvent for the water-insoluble polymer. As noted above, the poor solvent has a boiling point that is higher than that of the good solvent. When the solution is coated or cast onto a support and dried, the good solvent evaporates faster than the poor solvent, forming the membrane structure of the layer when the polymer phase separates from the solvent mixture. The open-pore structure results when the good solvent and poor solvent are removed by drying.

The water-insoluble polymer that can be used in the invention may be, for example, a cellulose ester such as cellulose diacetate, cellulose triacetate, cellulose acetate propionate or cellulose acetate butyrate, cellulose nitrate, polyacrylates such as poly(methyl methacrylate), poly(phenyl methacrylate) and copolymers with acrylic or methacrylic acid, or sulfonates, polyesters, polyurethanes, polysulfones, urea resins, melamine resins, urea-formaldehyde resins, polyacetals, polybutyrals, epoxies and epoxy acrylates, phenoxy resins, polycarbonates, vinyl acetate polymers and copolymers, vinyl chloride-vinyl acetate copolymers, vinyl chloride-vinyl acetate-vinyl-alcohol copolymers, vinyl chloride-vinyl acetate-maleic acid polymers, vinyl chloride-vinylidene chloride copolymers, vinyl chloride-acrylonitrile copolymers, acrylic ester-acrylonitrile copolymers, acrylic ester-vinylidene chloride copolymers, methacrylic ester-styrene copolymers, butadiene-acrylonitrile copolymers, acrylonitrile-butadiene-acrylic or methacrylic acid copolymers, or styrene-butadiene copolymers. Cellulose ester derivatives, such as cellulose diacetates and triacetates, cellulose acetate propionate, cellulose acetate butyrate, cellulose nitrate, and mixtures thereof are preferred.

The water-absorbent polymer that is used in the invention may be, for example, polyvinylpyrrolidone and vinylpyrrolidone-containing copolymers, polyethyloxazoline and oxazoline-containing copolymers, imidazole-containing polymers, polyacrylamides and acrylamide-containing copolymers, poly(vinyl alcohol) and vinyl-alcohol-containing copolymers, poly(vinyl methyl ether), poly(vinyl ethyl ether), poly(ethylene oxide), hydroxyethylcellulose, hydroxpropylcellulose, hydroxypropylmethylcellulose, methylcellulose, and mixtures thereof.

The choice of a good and poor solvent for the water-insoluble polymer will be effectively determined by the specific choice of polymer. The good solvent that can be used in the invention includes alcohols such as methanol, ethanol, n-propyl alcohol, isopropyl alcohol, isobutyl alcohol, Dowanol® solvents, glycols, ketones such as acetone, 2-butanone, 3-pentanone, cyclopentanone, and cyclohexanone, ethyl acetate, methylacetoacetate, diethylether, tetrahydrofuran, acetonitrile, dimethylformamide, dimethylsulfoxide, pyridine, chlorinated solvents such as methylene chloride, chloroform, carbon tetrachloride, and dichloroethane, hexane, heptane, cyclopentane, cyclohexane, toluene, xylenes, nitrobenzene, and mixtures thereof.

The poor solvent that can be used in the invention may be, for example, alcohols such as ethanol, n-propyl alcohol, isopropyl alcohol, isobutyl alcohol, 2-methyl-2,4-pentanediol, and Dowanol® solvents, glycols, ketones such as 2-butanone, 3-pentanone, cyclopentanone, and cyclohexanone, ethyl acetate, methylacetoacetate, diethylether, tetrahydrofuran, acetonitrile, dimethylformamide, dimethylsulfoxide, pyridine, chlorinated solvents such as carbon tetrachloride, and dichloroethane, hexane, heptane, cyclopentane, cyclohexane, toluene, xylenes, nitrobenzene, water, and mixtures thereof.

Since the image recording element may come in contact with other image recording articles or the drive or transport mechanisms of image recording devices, additives such as filler particles, surfactants, lubricants, crosslinking agents, matte particles and the like may be added to the element to the extent that they do not degrade the properties of interest.

Filler particles may be used in the open-pore membrane such as silicon oxide, fumed silica, silicon oxide dispersions such as those available from Nissan Chemical Industries and DuPont Corp., aluminum oxide, fumed alumina, calcium carbonate, barium sulfate, barium sulfate mixtures with zinc sulfide, inorganic powders such as γ-aluminum oxide, chromium oxide, iron oxide, tin oxide, doped tin oxide, alumino-silicate, titanium dioxide, silicon carbide, titanium carbide, and diamond in fine powder, as described in U.S. Patent 5,432,050.

A dispersing agent, or wetting agent can be present to facilitate the dispersion of the filler particles. This helps to minimize the agglomeration of the particles. Useful dispersing agents include, but are not limited to, fatty acid amines and commercially available wetting agents such as Solsperse® sold by Zeneca, Inc. (ICI). Preferred filler particles are silicon oxide, aluminum oxide, calcium carbonate, and barium sulfate. Preferably, these filler particles have a median diameter less than 1.0 µm. The filler particles can be present in the amount from 0 to 80 percent of the total solids in the dried open-pore membrane layer, most preferably in the amount from 0 to 40 percent.

The open-pore membrane layer may include lubricating agents. Lubricants and waxes useful either in the open-pore membrane layer or on the side of the element that is opposite the open-pore membrane layer include, but are not limited to, polyethylenes, silicone waxes, natural waxes such as carnauba, polytetrafluoroethylene, fluorinated ethylene propylene, silicone oils such as polydimethylsiloxane, fluorinated silicones, functionalized silicones, stearates, polyvinylstearate, fatty acid salts, and perfluoroethers. Aqueous or non-aqueous dispersions of submicron size wax particles such as those offered commercially as dispersions of polyolefins, polypropylene, polyethylene, high density polyethylene, microcrystalline wax, paraffin, natural waxes such as carnauba wax, and synthetic waxes from such companies as, but not limited to, Chemical Corporation of America (Chemcor), Inc., Michelman Inc., Shamrock Technologies Inc., and Daniel Products Company, are useful.

The open-pore membrane layer may include coating aids and surfactants such as nonionic fluorinated alkyl esters such as FC-430®, FC-431®, FC-10®, FC-171® sold by Minnesota Mining and Manufacturing Co., Zonyl® fluorochemicals such as Zonyl-FSN®, Zonyl-FTS®, Zonyl-TBS®, Zonyl-BA® sold by DuPont Corp.; other fluorinated polymer or copolymers such as Modiper F600® sold by NOF Corporation, polysiloxanes such as Dow Coming DC 1248®, DC200®, DC510®, DC 190® and BYK 320®, BYK 322®, sold by BYK Chemie and SF 1079®, SF1023®, SF 1054®, and SF 1080® sold by General Electric, and the Silwet® polymers sold by Union Carbide; polyoxyethylene-lauryl ether surfactants; sorbitan laurate, palmitate and stearates such as Span® surfactants sold by Aldrich; poly(oxyethylene-co-oxypropylene) surfactants such as the Pluronic® family sold by BASF; and other polyoxyethylene-containing surfactants such as the Triton X® family sold by Union Carbide, ionic surfactants, such as the Alkanol® series sold by DuPont Corp., and the Dowfax® family sold by Dow Chemical.

The open-pore membrane layer may include crosslinking agents, such as organic isocyanates such as tetramethylene diisocyanate, hexamethylene diisocyanate, diisocyanato dimethylcyclohexane, dicyclohexylmethane diisocyanate, isophorone diisocyanate, dimethylbenzene diisocyanate, methylcyclohexylene diisocyanate, lysine diisocyanate, tolylene diisocyanate, diphenylmethane diisocyanate; aziridines such as taught in U. S. Patent 4,225,665; ethyleneimines such as Xama-7® sold by EIT Industries; blocked isocyanates such as CA BI-12 sold by Cytec Industries; melamines such as methoxymethylmelamine as taught in U. S. Patent 5,198,499; alkoxysilane coupling agents including those with epoxy, amine, hydroxyl, isocyanate, or vinyl functionality; Cymel® crosslinking agents such as Cymel 300®, Cymel 303®, Cymel 1170®, Cymel 1171® sold by Cytec Industries; and bis-epoxides such as the Epon® family sold by Shell. Other crosslinking agents include compounds such as aryloylureas, aldehydes, dialdehydes and blocked dialdehydes, chlorotriazines, carbamoyl pyridiniums, pyridinium ethers, formamidinium ethers, and vinyl sulfones. Such crosslinking agents can be low molecular weight compounds or polymers, as discussed in U. S. Patent 4,161,407 and references cited.

The useful thickness range of the open-pore membrane layer used in the invention is from 1 µm to 100 µm, preferably from 2 µm to 50 µm.

In the present invention, the base support for the open-pore membrane layer of the recording element can be opaque resin coated paper, plain paper, coated paper, synthetic paper, or a transparent material, such as cellulose derivatives, e.g., a cellulose ester, cellulose triacetate, cellulose diacetate, cellulose acetate propionate, cellulose acetate butyrate; polyesters, such as polyethylene terephthalate, polyethylene naphthalate, poly-1,4-cyclohexanedimethylene terephthalate, polybutylene terephthalate, and copolymers thereof; polyimides; polyamides; polycarbonates; polystyrene; polyolefins, such as polyethylene or polypropylene; polysulfones; polyarylates; polyether imides; and mixtures thereof. The papers listed above include a broad range of papers, from high end papers, such as photographic paper to low end papers, such as newsprint.

The support used in the invention may employ an undercoat or an adhesive layer such as, for example, a vinylidene chloride-methyl acrylate-itaconic acid terpolymer or a vinylidene chloride-acrylonitrile-acrylic acid terpolymer. Other chemical adhesives, such as polymers, copolymers, reactive polymers or copolymers, that exhibit good bonding between the open-pore membrane layer and the support can be used. Other methods to improve the adhesion of the layer to the support include surface treatment such as by corona-discharge, plasma-treatment in a variety of atmospheres, UV treatment, etc, which is performed prior to applying the layer to the support.

The recording element of the invention can contain one or more conducting layers such as an antistatic layer to prevent undesirable static discharges during manufacture and printing of the image. This may be added to either side of the element. Antistatic layers conventionally used for color films have been found to be satisfactory, such as those in U.S. Patent 5,147,768. Preferred antistatic agents include metal oxides, e.g., tin oxide, antimony doped tin oxide and vanadium pentoxide. These antistatic agents are preferably dispersed in a film-forming binder.

The layers described above may be coated by conventional coating means onto a support material commonly used in this art. Coating methods may include, but are not limited to, wound wire rod coating, knife coating, slot coating, slide hopper coating, gravure coating, spin coating, dip coating, skim-pan-air-knife coating, multilayer slide bead, blade coating, curtain coating, multilayer curtain coating and the like. Some of these methods allow for simultaneous coatings of more than one layer, which is preferred from a manufacturing economic perspective if more than one layer or type of layer needs to be applied. The support may be stationary, or may be moving so that the coated layer is immediately drawn into drying chambers.

Ink jet inks used to image the recording elements of the present invention are well known in the art. The ink compositions used in ink jet printing typically are liquid compositions comprising a solvent or carrier liquid, dyes or pigments, humectants, organic solvents, detergents, thickeners, preservatives, and the like. The solvent or carrier liquid can be solely water or can be water mixed with other water-miscible solvents such as polyhydric alcohols. Inks in which organic materials such as polyhydric alcohols are the predominant carrier or solvent liquid may also be used. Particularly useful are mixed solvents of water and polyhydric alcohols. The dyes used in such compositions are typically watersoluble direct or acid type dyes. Such liquid compositions have been described extensively in the prior art including, for example, U.S. Patents 4,381,946; 4,239,543 and 4,781,758.

The following examples further illustrate the invention.

### Example 1 (Shows need for water-absorbent polymer)

### Preparation of Element 1

A homogeneous solution was prepared from 8 wt. % cellulose diacetate, CDA, (CA398-30, Eastman Chemical Company), 4 wt. % polyvinylpyrrolidone, PVP, (K25 from Aldrich Chemical Co.), 52.8 wt. % acetone (good solvent), and 35.2 wt. % 2-methyl-2,4,-pentanediol (poor solvent). The solution was metered to a slot-die coating apparatus and coated onto a plain paper support moving at a speed of 15 m/min. The coated support immediately entered the drying section of the coating machine to remove substantially all solvent components and form an image receiving element comprised of a microporous membrane. The thickness of the dry microporous membrane layer was measured to be 9 µm.

### Preparation of Element 2

This element was prepared and coated the same as Element 1 except that the CDA was 6 wt. %, the PVP was PVP-360 (Sigma-Aldrich Company) at 2 wt. %, the acetone was 55.2 wt. % and the 2-methyl-2,4,-pentanediol was at 36.8 wt. %.

### Preparation of Element 3

This element was prepared and coated the same as Element 1 except that the CDA was 6 wt. %, polyethyloxazoline, PEOx (Polysciences Inc.) was employed instead of PVP at 2 wt. %, the acetone was 59.8 wt. % and the 2-methyl-2,4,-pentanediol was at 32.2 wt. %.

### Preparation of Control Element C-1 (no water-absorbent polymer)

A homogeneous solution was prepared from 9 wt. % cellulose diacetate, CDA, (CA398-30, Eastman Chemical Company), 52.3 wt. % acetone (good solvent), and 38.7 wt. % 2-methyl-2,4,-pentanediol (poor solvent). This element was coated and dried as in Element 1.

### Preparation of Control Element C-2 (no water-absorbent polymer)

A homogeneous solution was prepared from 9 wt. % CDA (CA398-30), 3 wt. % poly(methyl methacrylate), PMMA, (Scientific Polymer Products, Inc), 50.6 wt. % acetone, and 37.4 wt. % 2-methyl-2,4,-pentanediol. The solution was coated onto a plain paper support using a calibrated coating knife, and dried to remove substantially all solvent components to form a microporous membrane.

### Preparation of Control Element C-3 (no water-absorbent polymer)

This element was prepared and coated the same as Control Element C-2 except that poly(vinyl acetate), PVAc, (Scientific Polymer Products, Inc.) was used instead of PMMA

### Printing

A cyan ink jet ink was prepared using a standard formulation with Direct Blue 199 as the dye. Using an Epson 200® ink jet printer, a series of square patches of varying dye density were printed onto the above elements. The density of each patch was read using an X-Rite 820® densitometer. The red channel density of the cyan patch at D-max (the highest density setting) is reported in the following Table 1:

**Table 1**

| Element | Polymers (Wt. Ratios) | D-max |
|---|---|---|
| 1 | CDA / PVP (67/33) | 1.5 |
| 2 | CDA / PVP (75/25) | 1.3 |
| 3 | CDA / PEOx (75/25) | 1.3 |
| Control C-1 | CDA (100) | 1.0 |
| Control C-2 | CDA / PMMA (75/25) | 0.6 |
| Control C-3 | CDA / PVAc (75/25) | 0.5 |

The above results show that the elements of the invention all had higher densities as compared to the control elements.

### Example 2 (Shows need for at least 25 wt. % water-absorbent polymer)

### Preparation of Element 4

This element was prepared the same as Element 1 except that the acetone was 50.6 wt. % and the 2-methyl-2,4,-pentanediol was at 37.4 wt. %. The solution was coated the same as Control C-2.

### Preparation of Element 5

This element was prepared and coated the same as Element 4 except that the CDA was 5 wt. %, the PVP was at 3 wt. %, the acetone was 52.9 wt. % and the 2-methyl-2,4,-pentanediol was at 39.1 wt. %.

### Preparation of Element 6

This element was prepared the same as Element 4 except that the CDA was 6 wt. %, the PVP was at 2 wt. %, the acetone was 59.8 wt. % and the 2-methyl-2,4,-pentanediol was at 32.2 wt. %. The element was coated the same as Element 1.

### Preparation of Element 7

This element was prepared and coated the same as Element 6 except that Polymer M-1 (see below) was added at 4 wt. %, the acetone was 52.8 wt. % and the 2-methyl-2,4,-pentanediol was at 35.2 wt. %.

### Preparation of Element 8

This element was prepared and coated the same as Element 4 except that the CDA was 6 wt. %, polymer M-2 (see below) was employed instead of PVP at 2 wt. %, the acetone was 55.2 wt. % and the 2-methyl-2,4,-pentanediol was at 36.8 wt. %.

### Preparation of Element 9

This element was prepared and coated the same as Element 8 except that the polymer M-2 (see below) was at 4 wt. %, the acetone was 54.0 wt. % and the 2-methyl-2,4,-pentanediol was at 36.0 wt. %.

### Preparation of Element 10

This element was prepared and coated the same as Element 1 except that the CDA was 6 wt. %, polymer M-1 (see below) was employed instead of PVP at 3 wt. %, the acetone was 52.3 wt. % and the 2-methyl-2,4,-pentanediol was at 38.7 wt. %.

### Preparation of Control Element C-4 (water-absorbent polymer less than 25 wt. %)

This element was prepared and coated the same as Element 4 except that the CDA was 9 wt. %, the PVP was at 2 wt. %, the acetone was 51.2 wt. % and the 2-methyl-2,4,-pentanediol was at 37.8 wt. %.

### Preparation of Control Element C-5 (water-absorbent polymer less than 25 wt. %)

This element was prepared and coated the same as Control Element C-4 except that the PVP was at 1 wt. %, the acetone was 51.8 wt. % and the 2-methyl-2,4,-pentanediol was at 38.2 wt. %.

### Preparation of Control Element C-6 (water-absorbent polymer less than 25 wt. %)

This element was prepared and coated the same as Element 10 except that the polymer M-1 (see below) was at 1.2 wt. %, the acetone was 53.4 wt. % and the 2-methyl-2,4,-pentanediol was at 39.4 wt. %.

### Printing

The above elements of Example 2 were printed the same as in Example 1, except that Elements 8-10 and Control Element 6 were printed on a Lexmark Z-51 Printer and an additional ink was used: a magenta ink containing Dye 6 from U.S. Patent 6,001,161. The following results were obtained:

**Table 2**

| Element | Polymers (Wt. Ratios) | Total wt. % water-absorbent polymer | Cyan D-max | Magenta D-max |
|---|---|---|---|---|
| 4 | CDA/PVP (67/33) | 33.3 | 1.5 | |
| 5 | CDA/PVP (62.5/37.5) | 37.5 | 1.3 | |
| 6 | CDA/PVP (75/25) | 25.0 | 1.3 | |
| 3 | CDA/PEOx (75/25) | 25.0 | 1.3 | |
| 7 | CDA/PVP/M-1 (50/17/33) | 50.0 | 1.4 | |
| 8 | CDA/M-2 (75/25) | 25 | 1.5 | 1.5 |
| 9 | CDA/M-2 (60/40) | 40 | 1.5 | 1.6 |
| 10 | CDA/M-1 (67/33) | 33 | 1.4 | 1.4 |
| Control C-4 | CDA/PVP (81.8/18.2) | 18.2 | 0.8 | |
| Control C-5 | CDA/PVP (90 /10) | 10.0 | 0.8 | |
| Control C-6 | CDA / M-1 (83/17) | 17 | 1.2 | 1.2 |

The above results show that the elements of the invention all had a higher D-max than the control elements with less than 25 wt. % water-absorbent polymer.

### Preparation of M-1

Compound M-1 is a water-absorbent polymer and is a random copolymer of 1-vinylimidazole and ethyl acrylate and was synthesized as follows. A 3-L three-necked, round-bottomed flask fitted with a mechanical stirrer, reflux condenser and nitrogen inlet, was charged with 1200 g of N,N-dimethylformamide, 193.8 g of 1-vinylimidazole, and 206.2 g of ethyl acrylate. The solution was sparged with dry nitrogen for 30 min, and then 2.0 g of 2,2'-azobis(isobutyronitrile) was added and the flask was immersed in a 60°C constant temperature bath under a slight positive pressure of nitrogen and stirred for 24 hr. The polymer was precipitated into diethyl ether, filtered, and dried in vacuo for several days, resulting in an off-white solid.

### Preparation of M-2

Compound M-2 is a water-absorbent polymer and is a random copolymer of 1-vinylimidazole and 1-vinylpyrrolidone and was synthesized as follows. A 1-L three-necked, round-bottomed flask fitted with a mechanical stirrer, reflux condenser and nitrogen inlet adapter, was charged with 320 mL of pH 7 buffer, 45 mL of isopropyl alcohol, 8.7 g of 1-vinylimidazole, and 82.5 g of 1-vinylpyrrolidone. This solution was sparged with dry nitrogen for 30 min, and then 0.67 g of 4,4'-azobis(4-cyanovaleric acid) was added. The flask was immersed in a 60°C constant temperature bath under a slight positive pressure of nitrogen and stirring begun. A solution of 40 mL of pH 7 buffer, 6 mL of isopropyl alcohol, 8.7 g of 1-vinylimidazole, and 0.67 g of 4,4'-azobis(4-cyanovaleric acid) was prepared in a similar way and pumped into the reaction flask over 210 min. The polymerization was allowed to proceed for a total of 7 hours. The polymer was then dialyzed in Membra Cel® tubing with a 12,000 - 16,000 molecular weight cutoff for 16 hours, and then freeze-dried, giving an off-white solid.

### Example 3 (Shows need for at least 25 wt. % water-absorbent polymer)

### Preparation of Element 11

This element was prepared the same as Element 1 except that the CDA was 6 wt. %, the PVP was at 2 wt. %, the acetone was 53.0 wt. % and the 2-methyl-2,4,-pentanediol was at 39.0 wt. %. The element was coated the same as Control Element C-2.

### Preparation of Element 12

This element was prepared the same as Element 3 except that the acetone was 53.0 wt. % and the 2-methyl-2,4,-pentanediol was at 39.0 wt. %. The element was coated the same as Control Element C-2.

### Printing and dye light stability testing

The above elements of Example 3 and Element 10 and Control Elements C-1 and C-6 were printed the same as in Example 1, except that a Lexmark Z51 ink jet printer was used, with a magenta ink jet ink prepared using a standard formulation with Dye 6 from U.S. Patent 6,001,161, and a yellow inkjet ink prepared using a standard formulation with Direct yellow 132 dye. The density of each patch was read using an X-Rite ® 820 densitometer.

The printed elements were then subjected to 2 weeks exposure to 50 Klux high intensity daylight. The density of each patch was read after the light exposure test using an X-Rite ® 820 densitometer. The % dye retention was calculated as the ratio of the density after the light exposure test to the density before the light exposure test. The results for magenta D-max and yellow D-max were as follows:

**Table 3**

| Element | Polymers (Wt. Ratios) | % dye retention magenta D-max | % dye retention yellow D-max |
|---|---|---|---|
| 11 | CDA/PVP (75/25) | 87.8 | 84.1 |
| 12 | CDA/PEOx (75/25) | 90.2 | 89.5 |
| 10 | CDA/M-1 (67/33) | 91.6 | 88.3 |
| Control C-1 | CDA (100) | 33.6 | 38.7 |
| Control C-6 | CDA/M-1 (83/17) | 91.6 | 53.6 |

The above results show that the elements of the invention all had greater dye lightfastness of the printed image for both magenta and yellow dyes than the control elements with less than 25 wt. % water-absorbent polymer.

### Example 4 (Shows varying proportions of good and poor solvent and proportion of water-absorbent to water-insoluble polymer)

### Preparation of Element 13

This element was prepared and coated the same as Element 1 except that the CDA was 6 wt. %, the PVP was at 2 wt. %, the acetone was 55.2 wt. % and the 2-methyl-2,4,-pentanediol, MPD, was at 36.8 wt. %.

### Preparation of Element 14

This element was prepared and coated the same as Element 13 except that acetone was 62.1 wt. % and the 2-methyl-2,4,-pentanediol was at 29.9 wt. %.

### Preparation of Element 15

This element was prepared and coated the same as Element 13 except that the CDA was 7.33 wt. %, the PVP was K30 (Aldrich Chemical Co.) at 3.67 wt. %, the acetone was 62.3 wt. % and the 2-methyl-2,4,-pentanediol was at 26.7 wt. %.

### Printing and evaluation

The above elements of Example 4 were printed the same as in Example 3, except that a cyan ink jet ink, prepared using a standard formulation with Direct Blue 199 as the dye, was also used. The red channel density (cyan), green channel density (magenta), and blue channel density (yellow) patches at D-max (the highest density setting) are reported in Table 4. The gloss of the top surface of the unprinted image receiving layer was measured using a BYK Gardner gloss meter at an angle of illumination/reflection of 60°. The results are related to a highly polished black glass with a refractive index of 1.567 that has a specular gloss value of 100. The following results were obtained:

**Table 4**

| Element | Polymers (Wt. Ratios) | Acetone / MPD | 60° gloss | Cyan D-max | Magenta D-max | Yellow D-max |
|---|---|---|---|---|---|---|
| 13 | CDA/PVP (75/25) | 60/40 | 38 | 1.4 | 1.3 | 1.3 |
| 14 | CDA/PVP (75/25) | 67.5/32.5 | 47 | 1.5 | 1.4 | 1.3 |
| 15 | CDA/PVP (67/33) | 70/30 | 65 | 1.7 | 1.6 | 1.5 |

The above results show that the surface gloss and printed image density of the elements of the invention can be controlled by varying the relative proportions of good and poor solvent for the water-insoluble polymer, as well as the proportion of water-absorbent to water-insoluble polymer within the confines of the invention.

## Claims

1. An ink jet recording element comprising a support having thereon an image-receptive layer capable of accepting an ink jet image comprising an open-pore membrane of a mixture of a water-insoluble polymer and a water-absorbent polymer, said mixture containing at least 25% by weight of said water-absorbent polymer, said image-receiving layer being made by dissolving the mixture of polymers in a solvent mixture, said solvent mixture comprising at least one solvent which is a good solvent for said water-insoluble polymer and at least one poor solvent for said water-insoluble polymer, said poor solvent having a higher boiling point than said good solvent, coating the dissolved mixture on said support, and then drying to remove approximately all of the solvents to obtain said open-pore membrane.

2. The element of Claim 1 wherein said water-insoluble polymer is a cellulose ester.

3. The element of Claim 2 wherein said cellulose ester is cellulose acetate, cellulose acetate butyrate or cellulose acetate propionate.

4. The element of Claim 1 wherein said water-absorbent polymer is polyvinylpyrrolidone, a vinylpyrrolidone-containing copolymer, an imidazole-containing polymer or copolymer, polyethyloxazoline or an oxazoline-containing copolymer.

5. The element of Claim 1 wherein said open-pore membrane also contains filler particles of silicon oxide, aluminum oxide, calcium carbonate, barium sulfate, barium sulfate/zinc sulfide or titanium dioxide.

6. The element of Claim 1 wherein said open-pore membrane also contains a crosslinking agent.

7. The element of Claim 1 wherein said open-pore membrane has a thickness of 2 µm to 50 µm.

8. The element of Claim 1 wherein said good solvent is a ketone, ethyl acetate or methylene chloride.

9. The element of Claim 1 wherein said poor solvent is an alcohol, a glycol, a xylene, cyclopentane, cyclohexane or water.

10. An ink jet printing method, comprising the steps of:
A) providing an ink jet printer that is responsive to digital data signals;
B) loading said printer with the ink jet recording element of claim 1;
C) loading said printer with an ink jet ink composition; and
D) printing on said ink jet recording element using said ink jet ink in response to said digital data signals.
